

## UNITED STATES PATENT OFFICE

2,027,998

## PERMANENT MAGNET CONTAINING NICKEL, ALUMINUM, COBALT, AND CHROMIUM

Tokushichi Mishima, Yodobashi-ku,  
Tokyo, Japan

No Drawing. Original application January 20, 1932, Serial No. 587,822. Divided and this application August 7, 1935, Serial No. 35,207. In Japan August 27, 1931

4 Claims. (Cl. 175—21)

This invention relates to a strong permanent magnet and forms a divisional from the copending application 587,822 filed January 20, 1932.

This permanent magnet contains the main elements iron, nickel and aluminium, with iron as basic element, nickel 5 to 40% and aluminium 7 to 20%; with the auxiliary elements cobalt 0.5 to 30%, chromium 1 to 5% with or without carbon from trace to 1.5%.

10 In said original application 587,822 it is described that a so-called "irreversible nickel steel" can be changed into a "reversible steel" by the addition of aluminium thereby obtaining a strong magnetic alloy. According to the invention it 15 has been found that the addition of a proper amount of other metals as auxiliary elements will further improve the magnetic properties as well as the tenacity and ductility of the permanent magnet and facilitate the mechanical 20 working of the magnet.

It is well known that the more minute the microstructure of the magnet steels is, the greater is the increase in the number of molecular magnets arranged irregularly at the boundaries 25 of the crystal grains so that consequently the coercive force and the residual magnetism also increase. This feature is gained by the addition of certain amounts of one or more auxiliary metals to the main elements iron, nickel and aluminium in the proportions herein given.

According to this invention it has been found 30 that an addition of cobalt and chromium in a proper amount also improves the magnetic properties of the steel and that in addition also the crystal grains of the steel are made minute and therefore the steel has better magnetic property and forgeability. The proportion for addition is: chromium 1 to 5% and cobalt 0.5 to 40%.

In this case also the number of the molecular magnets arranged irregularly at the boundary of the crystal grains is increased, and higher coercive force and stronger residual magnetism are obtained.

5 Actual examples for this case are given below:

| Chemical composition (percent) |        |                |               |        | Magnetic properties               |                                       |
|--------------------------------|--------|----------------|---------------|--------|-----------------------------------|---------------------------------------|
| Iron                           | Nickel | Alumin-<br>ium | Chro-<br>mium | Cobalt | Coercive<br>force (Hc)<br>(gauss) | Residual<br>magnetism<br>(Br) (gauss) |
| 62.5                           | 16.0   | 9.0            | 2.5           | 10.0   | 195                               | 10,000                                |
| 55.3                           | 14.0   | 8.0            | 2.5           | 20.0   | 200                               | 10,000                                |
| 58.8                           | 24.0   | 9.0            | 2.0           | 6.0    | 290                               | 9,800                                 |
| 52.3                           | 30.0   | 10.0           | 2.5           | 5.0    | 520                               | 9,500                                 |

10 In this case it is also noted that the presence of carbon of below 1.5% and/or a small amount of impurities does not materially affect the magnetic properties of the alloy.

15 I claim:

1. A permanent magnet comprising 5 to 40% nickel, 7 to 20% aluminium, 0.5 to 30% cobalt, 1 to 5% chromium and the remainder iron.

2. A permanent magnet comprising 5 to 40% nickel, 7 to 20% aluminium, 0.5 to 30% cobalt, 1 to 5% chromium and the remainder substantially iron.

3. A permanent magnet comprising 5 to 40% nickel, 7 to 20% aluminium, 0.5 to 30% cobalt, 1 to 5% chromium, from trace to 1.5% carbon and the remainder iron.

4. A permanent magnet comprising 5 to 40% nickel, 7 to 20% aluminium, 0.5 to 30% cobalt, 1 to 5% chromium, from trace to 1.5% carbon and the remainder substantially iron.

20 25 30 35 TOKUSHICHI MISHIMA.